

## UNITED STATES PATENT OFFICE

EMIL THEISZ, OF BUDAPEST, HUNGARY, ASSIGNOR TO EGYESÜLT IZZÓLÁMPA ÉS VILLA-  
MOSSAGI RÉSZVÉNYTÁRSASÁY, OF UJ-PEST, HUNGARY

## PLATED METAL BODY AND METHOD OF PRODUCING SAME

No Drawing. Application filed September 5, 1930, Serial No. 479,923, and in Hungary December 23, 1929.

My invention refers to the plating of metal and more especially to the production on metal bases of coatings consisting of compounds known under the trade name of tungsten and of molybdenum bronzes. The invention also includes the products obtained.

As is well known to those skilled in the art tungsten bronzes and molybdenum bronzes are compounds which were hitherto produced by reducing acid tungstates and acid molybdates, respectively, at high temperature. It is thus possible to produce for instance barium tungsten bronze  $\text{BaW}_4\text{O}_{12}$  or sodium molybdenum bronze  $\text{Na}_2\text{Mo}_5\text{O}_{15}$ . More detailed descriptions of these compounds can be found in many text books, for instance in Smithell's "Tungsten" (London 1926), p. 38-39, where tungsten bronzes are defined as having the constitution  $\text{R}_2\text{OWO}_{2n}\text{WO}_3$ , wherein R is an alkali-forming or an alkaline earth or similar metal, while n is an integer. Thus tungsten and molybdenum bronzes can be defined by the formula  $\text{R}_2\text{OXO}_{2n}\text{XO}_3$ , wherein X is tungsten or molybdenum.

According to the present invention coatings consisting of these and similar bronzes can be produced in a simple manner on any metallic body. According to the invention the metal body to be coated or plated is placed in a suitable solution of a tungsten or molybdenum compound and inserted in an electric circuit as cathode, whereupon the solution is subjected to electrolysis. According to the experiences hitherto made the electrolyzing of solutions of normal orthotungstates or orthomolybdates results in the production of tungsten oxides or molybdenum oxides of a low stage of oxidation. Thus for instance, when subjecting to electrolytical decomposition a solution, slightly acidulated with sulfuric acid or hydrochloric acid, of sodium orthomolybdate  $\text{Na}_2\text{MoO}_4$ , there is separated out at the cathode a molybdenum oxide  $\text{Mo}_2\text{O}_3 + \text{aq}$ .

I have now found that if a metal body is inserted as a cathode in a solution of a salt of meta—or polytungstic acid or meta—or polymolybdic acid, electrolytic decomposition will result in the formation of tungsten

bronzes or molybdenum bronzes. By suitably selecting and maintaining the conditions of operation, such as for instance the temperature and concentration of the solution and the cathodic current density, the electrolytic process can be conducted in such manner that the bronzes obtained are precipitated on the metal body forming the cathode in the form of a firmly adhering and altogether uniform coating.

This coating can be produced with particular advantage from solutions of the alkali metal salts and alkaline earth metal salts of meta—or polytungstic acid or meta—or polymolybdic acid. I prefer using watery solutions of barium meta-tungstate  $\text{BaW}_4\text{O}_{13} + 9\text{H}_2\text{O}$  or strontium meta-tungstate  $\text{SrW}_4\text{O}_{13} + 9\text{H}_2\text{O}$ . By simultaneously varying the concentration of the solutions and the cathodic current density bronze coatings of different thicknesses can be produced in the same period of time.

In practising my invention I may for instance proceed as follows:

## Example 1

A metal body which may for instance have a surface area of  $100 \text{ mm}^2$  is placed in a 70% solution of barium meta-tungstate heated to  $80^\circ \text{ C}$ . and inserted as cathode in an electrolytic circuit comprising an anode consisting of a precious metal. I now apply to the electrodes a voltage such that the intensity of the current flowing through the solution corresponds to  $D_k = 100$  milli amp. per  $\text{cm}^2$  of cathodic current. In the present example the electrolytical process is carried through with a current of 0, 1 amp. The electrolytical process results in the almost immediate formation of a blue coherent bronze coating. The metal body is now removed from the solution, rinsed with hot water and dried.

## Example 2

The metal body to be coated is placed in a solution of barium meta molybdate kept at ordinary temperature and inserted as cathode in a circuit traversed by an electric current having a cathodic current density 100

of 1-2 milli amp. per  $\text{cm}^2$ , any desired metal body forming the cathode. There results a gradually thickening blue coating of barium molybdenum bronze. After the lapse of 5 about 3 minutes the circuit is interrupted, the metal body is withdrawn, washed with distilled water and dried.

The solution from which the barium molybdenum bronze is precipitated can be 10 produced for instance in the following manner: a watery sodium meta molybdate solution is treated with a solution of  $\text{BaCl}_2$  to produce the corresponding barium meta molybdate, which is then suspended in distilled water, dilute hydrochloric acid being 15 added until the barium meta molybdate has been dissolved.

*Example 3*

20 The metal body to be coated is placed in a solution of strontium meta-tungstate having a specific density of 1,4 and inserted as cathode in the electrolytic circuit, any desired metal body, for instance a piece of tungsten, being used as anode. At ordinary 25 temperature a current corresponding to a cathodic current density of 250 milli amp. per  $\text{cm}^2$  is allowed to flow through the solution. As soon as a layer of the desired thickness has been deposited on the metal cathode 30 the current is interrupted, the metal body withdrawn, washed with hot water and dried.

I may also use mixtures of the different 35 salts.

The new method thus allows plating metal bodies of all descriptions, for instance bodies consisting of tungsten, molybdenum, platinum or nickel with one of these bronzes. 40 Owing to their advantageous properties the metal bodies plated in this manner are particularly adapted for the production of oxide cathodes.

Various changes may be made in the details disclosed in the foregoing specification 45 without departing from the invention or sacrificing the advantages thereof.

I claim:—

1. As a new product a metal body electroplated with a compound having the formula  $\text{R}_2\text{OXO}_{2n}\text{XO}_8$ , wherein X is tungsten or molybdenum, while R is an alkali-forming or an alkaline earth or similar metal and n is an integer. 50

2. As a new product a metal body electroplated with a compound having the formula  $\text{R}_2\text{OWO}_{2n}\text{WO}_8$ , wherein R is an alkali-forming or an alkaline earth or similar metal and n is an integer. 55

3. As a new product a metal body electroplated with a compound having the formula  $\text{R}_2\text{OMoO}_{2n}\text{MoO}_8$ , wherein R is an alkali-forming or an alkaline earth or similar metal and n is an integer. 60

4. As a new product a metal body electro-

plated with a compound having the formula  $\text{BaOWO}_{2n}\text{WO}_8$ , wherein n is an integer. 65

5. As a new product a metal body electroplated with a compound having the formula  $\text{BaMoO}_{2n}\text{MoO}_8$ , wherein n is an integer. 70

6. As a new product a metal body electroplated with a compound having the formula  $\text{SrOWO}_{2n}\text{WO}_8$ , wherein n is an integer. 75

7. The method of plating metal bodies comprising placing the body to be plated in a solution of a salt of the group of acids constituted by meta- or poly-tungstic and bodydic acids, inserting said body as cathode in an electric circuit and causing an electric current to act on the solution. 80

8. The method of plating metal bodies comprising placing the body to be plated in a solution of an alkali metal salt of the group of acids constituted by meta- or poly-tungstic and molybdc acids, inserting said body as cathode in an electric circuit and causing an electric current to act on the solution. 85

9. The method of plating metal bodies comprising placing the body to be plated in a solution of an alkaline earth metal salt of the group of acids constituted by meta- or poly-tungstic and molybdc acids, inserting said body as cathode in an electric circuit and causing an electric current to act on the solution. 90

In testimony whereof I affix my signature.  
EMIL THEISZ.

100

105

110

115

120

125

130

**CERTIFICATE OF CORRECTION.**

**Patent No. 1,896,022.**

**January 31, 1933.**

**EMIL THEISZ.**

It is hereby certified that the last word of the firm name of the assignee in the above numbered patent was erroneously described and specified as "Rész-venytársasay" whereas said last word should have been described and specified as "Részvénytársaság", as shown by the records of assignments in this office; and that the said Letters Patent should be read with this correction therein that the same may conform to the record of the case in the Patent Office.

Signed and sealed this 16th day of May, A. D. 1933.

**M. J. Moore.**

**(Seal)**

**Acting Commissioner of Patents.**